

## UNITED STATES PATENT OFFICE

FRANK S. WOOD, OF QUINCY, MASSACHUSETTS

## SAFETY PAPER

No Drawing.

Application filed April 22, 1931. Serial No. 532,115.

This invention relates to so called safety papers and to the process of preparing such papers so that when once written on with ink the writing cannot be removed, altered or re-  
 5 placed without setting the ink and leaving tell-tale stains, discolorations or alterations in the surface of the paper.

Such papers and treatments have heretofore been proposed but no ferrocyanide  
 10 treated paper has been produced which would not discolor with age or on exposure to light. Such discoloration previous to use of course rendered the paper unacceptable for most purposes and in fact such inherent discolora-  
 15 tion defeated the possibilities of detection of tampering by discolorations developed by ink eradicators. Ferrocyanide of potassium was proposed as an inkset by Dr. Ernest E. Schmidt in his Patent #1,217,076 of April  
 20, 1917 and as an inkset had a considerable effectiveness. Paper, however, so treated developed discoloration to such an extent that it proved unacceptable in use.

I have discovered that by giving the paper  
 25 a moderate alkalinity I can use ferrocyanide of potassium without discoloration of the paper while yet providing an ink set in the paper and making it possible to detect stains, spots, and other tell-tale signs where an ink  
 30 eradicator has been used.

In many commercial papers which are nor-  
 mally on the acid side in order to develop  
 35 an inkset which will not discolor when treated with such ink setting materials as ferrocyanide either of potassium or sodium, this acid condition of the paper must be neutralized and paper made moderately alkaline. The treatment varies according to different papers and their normal acid or alkaline con-  
 40 dition.

The alkaline condition in the paper does not in any way interfere with the inkset qual-  
 45 ities of the ferrocyanide solution but creates a condition in the paper whereby obvious evi-  
 dence of tampering with the original writing by ink eradicators results. I have discovered  
 50 that a paper of proper alkaline condition treated with an inkset will on the application of any known ink eradicator either develop a stain on the surface of the paper, or the spots

where the eradicator has been applied will be bleached to a degree which is readily ap-  
 parent.

While a great variety of formulæ are necessary in order to procure satisfactory  
 55 inksets in the several kinds of commercial paper, while simultaneously rendering the same subject to stain by the use of any chem-  
 60 ical intended to produce an eradication, it is important that a state of alkalinity suffi-  
 65 cient to prevent discoloration from the fer-  
 70 rocyanide treatment at all times be pro-  
 duced.

The different commercial papers in many instances have been treated with different  
 75 chemicals to produce the final finished arti-  
 80 cle and these chemicals have to be taken into consideration in determining the proper for-  
 85 mula of the inkset with which to treat any  
 90 one paper. If colored papers are used it  
 95 may also be necessary to vary the formulæ to take into account the chemical nature of  
 the coloring material.

For the purposes of my present invention  
 65 it is not believed to be necessary to set forth  
 70 these many formulæ, as my invention may  
 75 be practiced by producing a state of alka-  
 80 linity which will prevent discoloration,  
 85 while at the same time promptly showing an  
 90 inkset and stain upon the use of an ink  
 95 eradicator.

In checking the use of any particular com-  
 85 pound of any given paper, I dip a slip of  
 90 paper into the compound for an instant,  
 95 preferably not over two seconds of time, let  
 it dry and then write upon it with ink and  
 let that dry, then try to remove the writing  
 with ink eradicator. The acid of the ink  
 100 eradicator sets the ink while the chlorine  
 emphasizes it and causes a surface stain on  
 the paper. Frequently, chlorine will re-  
 move the inkset by destroying the surface of  
 the paper and soaking it through. When  
 the paper dries a yellow stain on the white  
 paper outlines where the surface has been  
 wet and the paper will be disfigured with  
 innumerable fine wrinkles. Although in  
 some cases those stains may be removed by  
 a solution of sodium bisulphate and the pa-  
 per restored to its white appearance, when,

however, the paper dries it will be noticed that wherever sodium bisulphite is applied the surface of the paper is whiter. If the paper is held up to the light a dark stain would be seen inside the paper, notwithstanding the fact that both surfaces appear whiter. This dark stain cannot be removed without destroying the paper.

Various modifications in the amount of alkaline may be employed as well as in the other chemicals used without departing from the spirit of my invention if within the limits of the appended claims.

What I therefore claim and desire to secure by Letters Patent is:

1. The method of producing a safety paper consisting in creating an alkaline state in such paper and in so treating said paper with a ferrocyanide as to produce an ink set condition without affecting the normal color of the paper.

2. The method of producing a safety paper consisting in creating an alkaline state in such paper by an acid neutralizing carbonate and in so treating said paper with a ferrocyanide as to produce an ink set condition without affecting the normal color of the paper.

3. The method of producing a safety paper consisting in creating an alkaline state in such paper by carbonate potassium or sodium and in so treating said paper with a ferrocyanide as to produce an ink set condition without affecting the normal color of the paper.

4. A safety paper treated with an alkali and a ferrocyanide in such proportions as to produce an ink set condition therein without affecting the normal color of the paper.

5. A safety paper treated with an alkali and a ferrocyanide in such proportions as to produce an ink set condition therein without affecting the normal color of the paper, said paper being of a nature to show discoloration when an ink eradicator is applied thereto.

6. A safety paper treated with such proportions of carbonate of potassium and ferrocyanide as to produce an ink set condition therein without affecting the normal color of the paper.

7. The method of producing a safety paper consisting in maintaining such paper sufficiently alkaline to neutralize ferrocyanide which is added thereto in quantity sufficient to produce an ink set condition therein but without destroying the normal color of the paper.

8. A safety paper treated with such proportions of carbonate of potassium and a ferrocyanide of potassium as to produce an ink set therein without affecting the normal color of the paper.

In testimony whereof I affix my signature.

FRANK S. WOOD.